

## UNITED STATES PATENT OFFICE

2,129,553

## TANNING MATERIAL

Alfred Russell and John W. Copenhaver, Philadelphia, Pa., assignors to Rohm & Haas Company, Philadelphia, Pa.

No Drawing. Application October 30, 1937,  
Serial No. 172,042

10 Claims. (Cl. 149—5)

This invention relates to the manufacture of tanning materials suitable for tanning pickled stock, for retanning leather already made by other means, and for bleaching or brightening chrome leather.

In our copending application, Serial No. 161,066, filed August 26, 1937, it is shown that excellent tanning materials especially suitable for the bleaching of chrome leather can be made by sulfonating a dihydroxy diaryl sulfone and condensing the resulting sulfone sulfonate with formaldehyde. We have now found that by co-condensing urea with the sulfone sulfonate and formaldehyde, a joint urea-sulfone sulfonate-formaldehyde condensate is obtained that has certain advantages over the material obtained from the sulfone sulfonate and formaldehyde only. These advantages are particularly noticeable when the new tanning materials are used to bleach chrome stock. A better bleaching and brightening is obtained and the leather has a greater resistance to the action of sunlight.

In practicing the invention the dihydroxy diaryl sulfone sulfonate prepared by any suitable method, as for instance those disclosed in the above mentioned copending application, is dissolved or diluted with water and to the solution urea is added and dissolved with the aid of heat if desired. The temperature of the solution is then raised to a point at which the urea and sulfone will react with formaldehyde and the formaldehyde added slowly. When all the formaldehyde has been added the temperature is maintained at or near the boiling point of the solution until reaction is complete. It may then be cooled, neutralized to the proper pH and diluted with water to the desired concentration.

The relative proportion of urea, sulfone sulfonate and formaldehyde that may be used varies over a wide range. The best ratio we have found is two molecular equivalents each of formaldehyde and sulfone sulfonate to one molecular equivalent of urea. These ratios we believe give on condensation a molecule having the formula



wherein the R's represent similar or dissimilar dihydroxy diaryl sulfone sulfonates attached to the methylene groups by nuclear carbon atoms. Reducing the quantity of urea decreases the quantity of this material in the final condensate but as the reaction product of sulfone sulfonate and formaldehyde is itself a tanning material, the tanning properties of the condensate are retained

and only the maximum advantage of the invention lost by the reduction. The formaldehyde may be reduced to a lower limit of one mol. of formaldehyde for each two mols of sulfone sulfonate particularly when less than the best ratio of urea to sulfonate is used. An excess over this lower limit equivalent to the quantity of urea used is desirable. A convenient rule to follow is to use at least one mol. of formaldehyde for each two mols of sulfone sulfonate plus one mol. of formaldehyde for each mol. of urea.

Increasing the quantity of urea and/or formaldehyde above the best ratios above mentioned leads to the formation of more complicated molecules that also have tanning properties but no further improvement is thereby obtained. However, if desired, up to four mols of formaldehyde and up to two mols of urea can be used with two mols of sulfone sulfonate.

The conditions of reaction such as temperature, dilution, acidity, etc., are largely a matter of choice and affect the speed of the reaction more than the quality of the reaction product. We prefer to carry out the reaction at or about the boiling point of water and at the natural pH of the sulfone sulfonate solution. Lower temperatures and high dilution slow the reaction and if the acidity becomes too high difficulty may be met in maintaining a suitably controlled rate of reaction. In the following examples, conditions of reaction we have found convenient are illustrated but by a few simple tests other conditions equally suitable can be readily determined. In these examples the parts given are by weight.

*Example 1.*—50 parts of 4:4' dihydroxy diphenyl sulfone is added to 70 parts of 98% sulfuric acid and the mixture heated at 110°—120° C. for from 15 to 20 minutes or until a product entirely soluble in water is obtained. The sulfonation mixture is cooled and diluted with 55 parts of water. 6 parts of urea are now added and the mixture heated to 98°—100° C. at which temperature all the urea dissolves readily. 17 parts 37% aqueous formaldehyde are now added slowly over ten minutes and the reaction mixture maintained at 98°—100° C. for four hours. It is then cooled somewhat, partly neutralized with 34 parts of caustic soda and diluted with water to a final mass of 520 parts.

*Example 2.*—50 parts of 4:4' dihydroxy diphenyl sulfone is sulfonated as in Example 1 using 70 parts of 98% sulfuric acid. 6 parts of urea is dissolved in the sulfonation mixture and 51 parts of water added. The mixture is then heated to 98°—100° C. and 20 parts of 30% aqueous

5 formaldehyde added slowly over 10 minutes. The mixture is maintained at 98°-100° C. and stirred continuously for three hours, then cooled, partly neutralized with 34 parts of caustic soda and diluted with water to a final mass of 520 parts.

10 The tanning materials produced as in these examples may be used alone or in combination with other tanning materials in tanning skins or in retanning leather made by other tanning materials but their greatest value is found in their ability to bleach and brighten chrome tanned leather. When used for this purpose they give a white leather that has a resistance to sunlight even greater than that produced from tanning 15 materials made from the sulfone sulfonate and formaldehyde alone. Other dihydroxy diaryl sulfone sulfonates such as those in which one or both the phenyl groups of the diphenyl compound are substituted by one or more methyl or other 20 alkyl groups may be substituted for the dihydroxy diphenyl sulfone sulfonate used in these examples.

25 In order to illustrate the use of these tanning materials to brighten chrome tanned leather the following example is given.

30 *Example 3.*—100 pounds of fully tanned chrome calfskin is drummed for an hour at 140° F. with 150 pounds of water and ten pounds, or other suitable quantity, of the tanning material prepared as described in Example 1. The stock is now washed with water till it shows a pH of 4-4½ when it may be oiled and finished in any recognized manner. The leather so produced has a white surface of remarkable resistance to the 35 action of strong sunlight.

35 We claim:

1. The process of preparing a synthetic tanning material which comprises co-condensing a dihydroxy diaryl sulfone sulfonate and urea with formaldehyde.

40 2. The process of preparing a synthetic tanning material which comprises co-condensing a dihydroxy diphenyl sulfone sulfonate and urea with formaldehyde.

3. The process of preparing a synthetic tan-

ning material which comprises co-condensing 4:4' dihydroxy diphenyl sulfone sulfonate and urea with formaldehyde.

4. The process of preparing a synthetic tanning material which comprises co-condensing 5 substantially two molecular equivalents of a dihydroxy diphenyl sulfone sulfonate and substantially one molecular equivalent of urea and substantially two molecular equivalents of formaldehyde.

10 5. A synthetic tanning material which in the acidic form consists of the joint condensation product of a dihydroxy diaryl sulfone sulfonate and urea with formaldehyde.

15 6. A synthetic tanning material which in the acidic form consists of the joint condensation product of a dihydroxy diphenyl sulfone sulfonate and urea with formaldehyde.

20 7. A synthetic tanning material which in the acidic form consists of the joint condensation 20 product of 4:4' dihydroxy diphenyl sulfone sulfonate and urea with formaldehyde.

25 8. A synthetic tanning material which in the acidic form consists of the joint condensation products of substantially two molecular equivalents of a dihydroxy diphenyl sulfone sulfonate and substantially one molecular equivalent of urea and substantially two molecular equivalents of formaldehyde.

30 9. In the process of making leather the improvement which comprises treating a chrome tanned leather with a joint condensation product of a dihydroxy diphenyl sulfone sulfonate, urea and formaldehyde.

35 10. In the process of making leather the improvement which comprises treating a chrome tanned leather with a joint condensation product of substantially two molecular equivalents of a dihydroxy diphenyl sulfone sulfonate, substantially one molecular equivalent of urea, and substantially two molecular equivalents of formaldehyde.

ALFRED RUSSELL.  
JOHN W. COPENHAVER.